

# UNITED STATES PATENT OFFICE.

HIRAM G. HICKS, OF WORCESTER, MASSACHUSETTS.

## HARDENING COMPOUND.

SPECIFICATION forming part of Letters Patent No. 372,619, dated November 1, 1887.

Application filed February 17, 1887. Serial No. 227,959. (No specimens.)

*To all whom it may concern:*

Be it known that I, HIRAM G. HICKS, a citizen of the United States, residing at Worcester, in the county of Worcester, in the State 5 of Massachusetts, have invented a new and useful Improvement in Hardening Compounds, of which the following is a specification.

This invention relates to a composition of matter to be used for hardening iron or steel. 10 To prepare ten pounds of my composition, I take yellow prussiate of potash, five pounds; red prussiate of potash, one-half pound; borax, three pounds; rosin, one and one-half pounds. These ingredients are to be thoroughly mingled 15 by agitation in a fine or granular state.

In using the above named composition the iron or steel is heated to the degree generally known as "cherry-red," and the compound is sprinkled on the iron or steel so heated. The 20 iron or steel, with the compound sprinkled upon it, is then put into the fire or heating-

space and kept there, free from draft, for about two minutes. The iron or steel is then withdrawn from the supply of heat and plunged into cold water.

By the use of this compound iron and steel 25 will become hardened and toughened.

What I claim as new, and desire to secure by Letters Patent, is—

A sprinkling composition for hardening and 30 toughening heated iron and steel, consisting of yellow prussiate of potash, red prussiate of potash, borax, and rosin, in or about the proportions set forth, for the purposes specified.

In testimony whereof I have hereunto set 35 my hand and seal in the presence of two subscribing witnesses.

HIRAM G. HICKS. [L. s.]

Witnesses:

DAVID W. GOODRICH,  
E. F. KASTENHUBER.